

## UNITED STATES PATENT OFFICE.

ARMAND DE WAELE, OF LONDON, ENGLAND, ASSIGNOR TO D. GESTETNER, LIMITED, OF LONDON, ENGLAND.

PRODUCTION OF STENCILS FOR USE IN DUPLICATING MANUSCRIPT AND TYPE-WRITTEN DOCUMENTS, DRAWINGS, AND THE LIKE.

No Drawing. Application filed October 23, 1924, Serial No. 745,496, and in Great Britain October 29, 1923.

This invention relates to the production of stencils for use in duplicating manuscript and typewritten documents, drawings and the like and particularly stencils of the type in which a porous support, such as yoshino paper, is provided with a stencil layer including a gelatinized organic colloid which does not need moistening in order to soften the coating composition prior to cutting the stencil.

The employment of colloids of vegetable origin free from nitrogen as, for instance, Irish moss in association with gelatine has been proposed in the production of the composition forming the stencil layer but it has been indicated that glycerine should be employed in conjunction therewith as the sole tempering agent in order to obtain stencil sheets which do not need moistening prior to cutting.

The use of glycerine in such proportions that the stencil sheet may be cut without previous moistening is however open to objection owing to its hygroscopicity but mainly because the mechanical properties of the stencil layer are unsatisfactory.

The present invention consists, broadly, in a stencil sheet in which the ink-resisting medium of the stencil comprises a gelatinized sea-weed jelly, such as agar-agar, Iceland moss, Irish moss, carragheen moss, Japanese isinglass and the like or other gelatinizing carbohydrate or gelatinizing organic colloids derived from such bodies in combination with a tempering agent which is not hygroscopic and does not contain water.

The invention consists more particularly in a stencil sheet comprising a gelatinized sea-weed jelly and an oleaginous or waxy material acting as tempering agent.

Preferably, the oily or waxy bodies employed are soft or even liquid at the ordinary temperature of the air and if necessary they are employed in association with an agent adapted to secure their emulsification in the organic colloid disperse.

Preferably, as emulsifying agents, sulphonated fats or waxes and particularly sulphonated fats or liquid waxes or products containing material proportions of liquid waxes derived from marine animals are employed.

Thus, in accordance with the invention

sulphonated sperm oil may be used as the emulsifying agent and it may also act as 65 tempering agent.

Preferably the sulphonated sperm oil or other emulsifying agent is employed in association with an unsulphonated oil, for instance light mineral oil.

The oily or waxy constituents are present in the stencil layer in accordance with the invention in such proportion that they constitute wholly or mainly the tempering agent for the organic colloid, for instance, agar-agar, that is to say, the agent adapted so to modify the properties of the colloid that the structure of the stencil layer may be broken down by the blows of the type when used in forming stencils in a typewriter or by the stile when producing a stencil by hand.

In addition to oily or waxy constituents or other bodies which are not hygroscopic or do not contain water, a small proportion of hygroscopic or water-containing bodies may be present in the stencil layer. Thus for instance, a small quantity of glycerine may be present therein and in such case the glycerine or the equivalent may merely operate to render more flexible the gelatinous structure through which the material functioning as the tempering agent is dispersed.

The proportion of the tempering agent I have found it convenient to employ may vary between six or ten parts to one of a colloid. This indication, however, is only given for the purpose of illustrating the proportion I have found it convenient to use in certain atmospheric or climatic conditions.

Conveniently, inorganic materials may be incorporated in the composition as indicated in the complete specification of the application for British Letters Patent No. 27,074 of 1923. Thus for instance the material known as "bentonite" may be included in the composition.

Also an opaque pigment, the colour of which will contrast with the ink with which the stencil will be used, for instance, a white pigment, may be incorporated in the stencil layer as indicated in the specification of the application for British Letters Patent No. 29,406 of A. D. 1922, care being taken

to select a pigment which does not operate to break down the structure of the coating composition.

In forming the stencil composition, it may be convenient to omit the emulsifying agent, in which case it may be desirable or even necessary to employ mechanical means for securing the dispersion of the tempering agent as specified in the specification of the application for British Letters Patent No. 27,073 of 1923.

The invention also extends to a method of effecting the dispersion of the sea-weed jellies and other gelatinizing organic colloids employed in the production of stencil sheets as described by subjecting the same with or without preliminary soaking or swelling, together with the dispersion medium, to mechanical treatment adapted to secure its division into particles of ultra-microscopic fineness.

As indicative of the treatment contemplated, it may be remarked that the organic colloid and the disperse medium may be passed together between surfaces spaced apart about 0.007 of an inch and moving relatively to one another at the rate of 17,000 to 18,000 feet per minute.

Thus, in order to secure the desired degree of dispersion a device comprising discs, the faces of which are spaced 0.007 inch apart, fourteen inches in diameter and rotated relatively to one another at a speed of 5,000 revolutions per minute, may be employed.

The immediate effect to be secured is similar to that secured in homogenizing milk, the ultimate result being similar also.

The mechanical treatment to which the mixture of colloid and disperse medium is subjected will raise its temperature and to some extent this may assist in securing the solution of the colloid; the rise in temperature will, however, be quite insufficient in itself to effect solution of a material such as agar-agar.

With agar-agar or Irish moss or other sea-weed jellies after the mixture thereof and water has been subjected to mechanical treatment of the character indicated it is merely necessary to raise the temperature of the product to 90° C. or thereabouts in order to obtain a satisfactory sol.

When the sol has been formed in this or any other convenient manner the tempering agent is incorporated in it.

In conclusion it may be pointed out that the scope of the invention is not to be regarded as limited to the employment of the specific examples of gelatinizing organic colloids given herein but extends to the employment of all suitable bodies falling within the ambit of the generic terms irrespective of whether these bodies occur in nature in a suitable form or are prepared artificially.

Having now described my invention,

what I claim as new and desire to secure by Letters Patent is:—

1. A stencil sheet adapted to be stencil-  
ized by pressure, comprising a highly porous support and a substantially non-hygroscopic ink-resisting coating thereon including a gelatinizing carbohydrate in combination with a tempering agent which is not hygroscopic and does not contain a material proportion of water, said tempering agent being present in sufficient quantity to enable the sheet to be stencilized in a substantially dry state. 75

2. A stencil sheet adapted to be stencil-  
ized by pressure, comprising a highly porous support and a coating thereon of an ink-  
resisting medium including a gelatinizing carbohydrate and an oleaginous material acting as the main tempering agent. 80

3. A stencil sheet adapted to be stencil-  
ized by pressure, comprising a highly porous support and an ink-resisting coating thereon including a gelatinizing carbohydrate and a proportion of an oleaginous non-hygroscopic material adapted to render the coating suf-  
ficiently sensitive for stencilization in a sub-  
stantially dry state. 85 90

4. A stencil sheet adapted to be stencil-  
ized by pressure, comprising a highly porous support, a coating thereon of an ink-resist-  
ing medium substantially free from water,  
consisting essentially of a gelatinizing car-  
bohydrate, an oleaginous non-hygroscopic  
material adapted to render the coating suf-  
ficiently sensitive for stencilization in a 100  
substantially anhydrous condition and an  
agent adapted to secure the emulsification  
of the oleaginous material in the gelatiniz-  
ing carbohydrate. 105

5. A stencil sheet adapted to be stencil-  
ized by pressure, comprising a highly porous support, a coating thereon of an ink-resist-  
ing medium including a gelatinizing carbo-  
hydrate and an oleaginous material adapted  
to render the coating sufficiently sensitive 110  
for stencilization in the absence of moisture,  
and a sulphonated oil derived from a marine  
animal adapted to secure the emulsification  
of the oleaginous material in the gelatiniz-  
ing carbohydrate. 115

6. A stencil sheet adapted to be stencilized  
by pressure, comprising a highly porous sup-  
port, a coating thereon of an ink-resisting  
medium consisting essentially of a gelatiniz-  
ing carbohydrate, an oleaginous non-hy-  
groscopic material in a proportion adapted  
to render the coating sufficiently sensitive  
for stencilization when free from moisture  
and sulphonated sperm oil as the agent  
adapted to emulsify the oleaginous material 125  
in the carbohydrate. 120

7. A stencil sheet adapted to be stencil-  
ized by pressure, comprising a highly porous support and a coating thereon of an ink-  
resisting medium including a gelatinizing 130

- carbohydrate, an oleaginous non-hygroscopic material acting as the main tempering agent and present in the medium in a proportion considerably in excess of the 5 proportion of gelatinizing carbohydrate therein, and a small proportion of hygroscopic or water-containing bodies in a proportion operating to render more flexible the gelatinous structure through which the 10 material functioning as the tempering agent is dispersed.
8. A stencil sheet adapted to be stencilized by pressure, and in a substantially anhydrous state, comprising a highly porous 15 support and an ink-resisting coating thereon including a gelatinized seaweed jelly in combination with a tempering agent which is not hygroscopic and does not contain a material proportion of water.
- 20 9. A stencil sheet adapted to be stencilized by pressure, comprising a highly porous support and a coating thereon of an ink-resisting medium including a gelatinized seaweed jelly and an oleaginous material 25 acting as tempering agent in sufficient proportion to enable the stencil sheet to be stencilized when substantially free from water.
10. A stencil sheet adapted to be stencilized by pressure, comprising a highly porous support and an ink-resisting coating thereon substantially free from water, including a gelatinized seaweed jelly and a 30 proportion of an oleaginous material adapted 35 to render the coating sufficiently sensitive for stencilization without moistening.
11. A stencil sheet adapted to be stencilized by pressure, comprising a highly porous support, a coating thereon of an ink-resisting medium including a gelatinized 40 seaweed jelly and an oleaginous material in a proportion considerably in excess of the proportion of seaweed jelly adapted to render the coating sufficiently sensitive for 45 stencilization in a substantially dry state and an agent adapted to secure the emulsification of the oleaginous material in the gelatinized seaweed jelly.
12. A stencil sheet adapted to be stencilized by pressure, comprising a highly porous support, a coating thereon of an ink-resisting medium including a gelatinized seaweed jelly, an oleaginous material adapted 50 to render the coating sufficiently sensitive for stencilization in the absence of added moisture, and a sulphonated oil derived from a marine animal adapted to secure the emulsification of the oleaginous material in the gelatinized seaweed jelly.
- 55 13. A stencil sheet adapted to be stencilized by pressure, comprising a highly porous support, a coating thereon of an ink-resisting medium including a gelatinized seaweed jelly, an oleaginous material adapted 60 to render the coating sufficiently sensitive for stencilization in the absence of added moisture, and a sulphonated oil derived from a marine animal adapted to secure the emulsification of the oleaginous material in the gelatinized seaweed jelly.
- 65 14. A stencil sheet adapted to be stencilized by pressure, comprising a highly porous support and a coating thereon of an ink-resisting medium including a gelatinized seaweed jelly and an oleaginous material 70 acting as tempering agent in a proportion many times greater than the proportion of seaweed jelly, and a small proportion of hygroscopic or water-containing bodies in a proportion operating to render more flexible the gelatinous structure through which the material functioning as 75 the tempering agent is dispersed.
15. A stencil sheet adapted to be stencilized by pressure, comprising yoshino paper and an ink-resisting coating thereon including a gelatinizing carbohydrate and an oleaginous material adapted to render the coating sufficiently sensitive for stencilization in a substantially air-dry state.
16. A stencil sheet adapted to be stencilized by pressure, comprising yoshino paper, a coating thereon of an ink-resisting medium including a gelatinizing carbohydrate, an oleaginous material adapted to render the coating sufficiently sensitive for stencilization in a substantially dry state and an agent adapted to secure the emulsification of the oleaginous material in the gelatinizing carbohydrate. 80
17. A stencil sheet adapted to be stencilized by pressure, comprising yoshino paper, a coating thereon of an ink-resisting medium including a gelatinizing carbohydrate and an oleaginous material adapted to render the coating sufficiently sensitive for stencilization in a proportion considerably exceeding the proportion of the carbohydrate, and a sulphonated oil derived from a marine animal adapted to secure the emulsification of the oleaginous material in the gelatinizing carbohydrate. 85
18. A stencil sheet adapted to be stencilized by pressure, comprising yoshino paper, a coating thereon of an ink-resisting medium including a gelatinizing carbohydrate, an oleaginous material adapted to render the coating sufficiently sensitive for stencilization in a substantially dry state and sulphonated sperm oil as the agent adapted to emulsify the oleaginous material in the carbohydrate. 90
19. A stencil sheet adapted to be stencilized by pressure, comprising yoshino paper and a coating thereon of an ink-resisting medium including a gelatinizing carbohydrate, an oleaginous material acting as the main tempering agent present in the coating in a proportion many times greater than the proportion of carbohydrate therein, and a small proportion of hygroscopic or water-containing bodies in a proportion operating to render more flexible the gelatinous structure through which the material functioning as the tempering agent is dispersed. 95
- 100
- 105
- 110
- 115
- 120
- 125
- 130

to render more flexible the gelatinous structure through which the material functioning as the tempering agent is dispersed.

20. A stencil sheet adapted to be stencilized by pressure, comprising yoshino paper and a coating thereon of an ink-resisting medium including a gelatinized seaweed jelly and a proportion of an oleaginous material acting as tempering agent many times greater than the proportion of seaweed jelly.

21. A stencil sheet adapted to be stencilized by pressure, comprising yoshino paper and an ink-resisting coating thereon including a gelatinized seaweed jelly and an oleaginous material adapted to render the coating sufficiently sensitive for stencilization in a substantially air-dry state.

22. A stencil sheet adapted to be stencilized by pressure, comprising yoshino paper, a coating thereon of an ink-resisting medium including a gelatinized seaweed jelly, a proportion of an oleaginous material adapted to render the coating sufficiently sensitive for stencilization in a substantially dry state and a sulphonated oil derived from a marine animal adapted to secure the emulsification of the oleaginous material in the gelatinized seaweed jelly.

23. A stencil sheet adapted to be stencilized by pressure, comprising yoshino paper and a coating thereon of an ink-resisting medium including a gelatinized seaweed jelly and a proportion of an oleaginous material acting as tempering agent many times greater than the proportion of seaweed jelly, and a small proportion of hygroscopic or water-containing bodies in a

proportion operating to render more flexible the gelatinous structure through which the material functioning as the tempering agent is dispersed.

24. A stencil sheet comprising a base of open porous material coated with a composition substantially free from water and hygroscopic materials, consisting essentially of a gelatinized carbohydrate deposited from an aqueous medium and a fatty acid ester of high molecular weight and of an oleaginous character, said ester being present in a proportion sufficient to maintain the composition permanently in a state in which it may be stencilized when substantially free from moisture.

25. A stencil sheet comprising a base of open porous material coated with a composition consisting essentially of an emulsion of a gelatinized carbohydrate deposited from an aqueous medium and an oleaginous fatty acid ester in a proportion sufficient to maintain the composition permanently in a state in which it may be stencilized when substantially free from moisture.

26. A stencil sheet comprising a base of open porous material coated with a composition consisting essentially of an emulsion of a gelatinized carbohydrate and an oleaginous fatty acid ester in a proportion sufficient to maintain the composition permanently in a state in which it may be stencilized when substantially free from moisture.

In testimony whereof I have signed my name to this specification.

ARMAND DE WAELLE.